

## UNITED STATES PATENT OFFICE

2,002,523

## PROCESS OF PREVENTING CORROSION

Hyym E. Buc, Roselle, N. J., assignor to Standard  
Oil Development Company, a corporation of  
Delaware

No Drawing. Application July 23, 1932,  
Serial No. 624,361

10 Claims. (Cl. 252—5)

This invention relates to a process for preventing corrosion of metals in contact with acid alkaline or neutral aqueous mediums and will be fully understood from the following description:

5 Two beakers of dilute acetic acid are taken and a piece of copper wire placed in each. To one of the beakers a small amount of tertiary amyl phenol is added. After letting the beakers stand several weeks exposed to the air the solution containing no amyl phenol turns blue while the other remains water white. In this case the tertiary amyl phenol evidently prevents the acid corrosion of the copper wire.

Extending the scope of this preliminary experiment I have found that the corrosion of other metals in acid alkaline or neutral aqueous mediums can be prevented or considerably decreased by the addition of small amounts of corrosion preventatives of the phenol type and belonging generally to the class of substances consisting of phenols, naphthols, alkylated phenols, alkylated naphthols, and the sulfonated derivatives of these various phenolic compounds.

The expression "phenol" is meant to comprise both mono and polyhydric phenols. Phenolic substances containing other groups besides the hydroxyl such as, for example, amino phenols, may also be used although the phenols and alkylated phenols containing no such additional group in the ring are preferred.

The expression "aqueous medium" is to be taken in a broad sense so as to cover cases when the water is present in solution or even only in traces, for example, it is usual to spray coal with 35 calcium chloride solution to prevent dust formation. In this case the aqueous medium is only present in traces forming a film over the surface of the coal particles, yet a serious corrosion of the equipment handling such treated coal has 40 been observed. Such corrosion is considerably reduced by the addition of my corrosion preventative substances to the calcium chloride solution before the spraying.

The corrosion of metals may be due to several causes. The main types of corrosion known are the oxidation corrosion and the electrolytic corrosion. I have found that the inhibitors belonging to the above described class of substances are active with the various types of cor- 45 osions although they are most frequently used with the oxidation type. When sulfonated derivatives are employed the same are most conveniently introduced in the form of neutral salts. Alkaline solutions are generally preferred for the 50 non-sulfonated phenols and naphthols, alkylated

phenols and alkylated naphthols, particularly to prevent metal corrosion due to oxidation.

The following experimental technique was developed for testing the efficiency of the corrosion inhibitors: weighed strips of different metals, the surface of which has been measured were left in contact with the aqueous medium for seven days at a temperature of 160° F. The metal strips were then taken out, washed, dried and weighed and their loss or gain of weight was calculated as corrosion over their total surface expressed in fractions of an inch of penetration per year. A loss of weight was designated as positive penetration while a gain of weight as negative penetration. It will be readily understood that both positive and negative penetration are due to corrosion. Positive penetration is shown, for example, by copper, while aluminum suffers negative penetration, that is, gain of weight. In the absence of corrosion there is, of course, no change in the weight of the metal strip. The corrosion in the presence of the corrosion inhibitor was then compared with the corrosion in the blank runs.

The corrosion in various mediums was studied by the above described method. The following examples will illustrate the action of my corrosion inhibitors:

0.5% of slightly alkaline solution of tertiary butyl phenol reduces a corrosion in a 29% calcium chloride solution by the following amounts:

|                            | Percent |
|----------------------------|---------|
| Copper                     | 50      |
| Brass                      | 50      |
| Iron                       | 33      |
| Solder (50% lead, 50% tin) | 87      |

All these metals suffer positive penetration. The corrosion of tin and aluminum by calcium chloride solutions of the same strength is reduced by 70% by the addition of 1/2% sodium tertiary butyl sulfonate; hydroquinone is somewhat less active. Alpha naphthol was found to efficiently reduce the corrosion of steel in 50% solutions of triethanolamine.

Glycerin solutions containing water, alcohol and castor oil are used for certain technical purposes, such as for example, radiator solutions for the cooling systems of internal combustion engines. The use of my corrosion inhibitors resulted in a reduction of 60 to 100% of the corrosion caused by such solutions on brass and solder.

Several of the solutions described, such as the calcium chloride solution and the glycerine solu-

tion referred to, are commonly classed together as anti-freeze solutions.

My corrosion inhibitors may be used in combination with other types of corrosion inhibitors 5 with very good results. Thus, for example, the corrosion of iron is greatly decreased in the presence of small amounts of a mixture of urea and phenol dissolved in the aqueous medium.

The amount of the corrosion inhibitor may 10 vary within considerable limits. Usually 0.1-0.5% of an inhibitor calculated on the amount of the neutral acid or alkali aqueous medium is sufficient for good results. Sometimes smaller amounts will do and sometimes larger amounts 15 have to be used. In general the amount of the inhibitor used is seldom outside the limits of 0.02-1%.

The inhibitors have to be brought in solution 20 in the aqueous medium, which is usually easily achieved. The phenolic inhibitor may, if necessary, be first dissolved in a small amount of alkali solution and then added to the aqueous medium.

The invention is not to be limited by any 25 theory nor by the examples given by way of illustration but only by the appended claims in which it is my intention to claim all novelty inherent in the invention.

I claim:

1. The process of decreasing the corrosion of 30 a metal in contact with an aqueous medium which comprises adding to the medium a small amount of an alkylated phenol as corrosion inhibitor.

2. The process of decreasing the corrosion of

a metal in contact in an aqueous medium which comprises adding to the medium a small amount of an alkylated aromatic compound of the group consisting of alkylated phenols and alkylated naphthols.

3. The process according to claim 2 in which 5 alkylated phenols are used.

4. The process according to claim 2 in which alkylated naphthol is used.

5. The process according to claim 1 in which 10 the corrosion inhibitor is added in an amount of 0.02-1%.

6. The process of decreasing the corrosion of 15 radiator solutions used for the cooling systems of internal combustion engines, which comprises adding to such solutions a small amount of an alkylated phenol as corrosion inhibitor.

7. The process of decreasing the corrosive action 20 of aqueous anti-freeze solutions, which comprises adding thereto from 0.2 to 1% of an alkylated phenol.

8. The process of decreasing the corrosion of 25 metals in contact with an aqueous medium, which comprises dissolving an alkylated phenol in a small amount of alkali solution and adding said solution to said aqueous medium.

9. An anti-freeze composition comprising a water-soluble anti-freeze compound and a small amount of an alkylated phenol.

10. An anti-freeze composition comprising a 30 water-soluble anti-freeze compound and a small amount of an alkylated naphthol.

HYYM E. BUC.